

1

3,070,473

## LIQUID PROPELLANTS

Ronald A. Henry, China Lake, Calif., and Charles W. Tait, Wyandotte, Mich., assignors to the United States of America as represented by the Secretary of the Navy  
No Drawing. Filed Nov. 1, 1957, Ser. No. 694,056

6 Claims. (Cl. 149—89)

(Granted under Title 35, U.S. Code (1952), sec. 266)

The invention described herein may be manufactured and used by or for the Government of the United States of America for governmental purposes without the payment of any royalties thereon or therefor.

This invention relates to new liquid monopropellant formulations derived from nitroalkanes.

Two of the disadvantages connected with the use of certain monopropellants, such as nitromethane, are that they are difficult to ignite and their burning rates are not particularly high. Nitromethane, for example, requires a high chamber pressure for its ignition and smooth, steady burning. High burning rates in the region of useful rocket pressures are desirable in the interest of increased thrust.

It is possible to obtain better ignitability and smoothness of burning by using hypergolic bipropellant systems, such as, hydrazine-nitric acid systems, but such systems in a rocket are mechanically more complicated than that required for a simple monopropellant. The smooth ignition and burning of nitromethane at low pressures (300—800 p.s.i.a.) can be accomplished by injecting small amounts of oxygen into the combustion chamber but this method is essentially a bipropellant system and possesses the mechanical problems associated with such systems. For example, all the difficulties inherent in handling compressed or liquid oxygen are retained.

It is therefore an object of this invention to provide a method for improving the ignitability and burning rate of liquid monopropellants without prohibitively altering their stability or calorific value.

It is another object of this invention to provide liquid monopropellant formulations ignitable at low chamber pressures and having increased burning rates.

It has been found that the above objects are accomplished by the addition to the monopropellant of up to about ten percent of an ultraviolet light absorber. The light absorbers found suitable are certain hydroxy-substituted benzophenones. While the explanation of the surprising effect produced by these additives is not definitely known, it is believed to be due to an increase in the amount of sub-surface reaction or decomposition produced by them.

The invention is illustrated by the following examples but is not limited thereby.

## Example I

A mixture of 2,2'-dihydroxy-4,4'-dimethoxybenzophenone and 2,2',4,4'-tetrahydroxybenzophenone was dissolved in nitromethane at a concentration level of about two percent by weight. Strands were made from the formulation and the strand burning rate determined in 4 mm. inside diameter glass tubes over the pressure range 750—1900 p.s.i.g. by the procedure of Tait, Williams and Whittaker, Journal of American Rocket Society, volume 85, page 83 (1951). This method was used in all examples set forth in this specification. The burning rate was about ten percent faster than that for nitromethane without the additive. More significantly, the pressure at which ignition and smooth burning occurred was lowered from about 1250—1300 p.s.i.g. for nitromethane alone to 775—800 p.s.i.g. for the mixture. The experiment was repeated with both five percent and ten percent by weight of the additive mixture with substantially the same results. The

2

limit of solubility of the additive mixture in nitromethane is slightly over ten percent. These results indicate that only small quantities of the ultraviolet light absorber are needed to effect very profound changes in the properties of the propellant.

## Example II

2,4-dihydroxybenzophenone was dissolved in nitromethane at a concentration level of two percent by weight; strands were made from the composition and the strand burning rate determined. An increase in burning rate of 10—20 percent resulted throughout the range of 1300—2100 p.s.i.g. Smooth burning was attained at a pressure of 700 p.s.i.g. Ten percent of 2,4-dihydroxybenzophenone added to nitromethane did not further lower this pressure but it did increase the burning rate another 5—10 percent.

In order to test the effectiveness of the ultraviolet light absorbers on nitric acid systems it was first necessary to nitrate them as they cannot be added to a nitric acid system without reacting and causing some reduction in nitric acid concentration. Although the ultraviolet light absorbers would be operative in the unnitrated form it is preferable to nitrate them before use. Two polynitro 2,4-dihydroxybenzophenones were synthesized as described below.

3,5-dinitro-2,4-dihydroxybenzophenone was prepared as follows: Three grams of 2,4-dihydroxybenzophenone, 60 ml. of 4 N nitric acid solution, and a trace of sodium nitrite were mixed and allowed to stand at room temperature for eight days. The mixture was shaken occasionally. Although the 2,4-dihydroxybenzophenone did not dissolve, it gradually changed color from white to pink. The solid was removed by filtration, washed with cold water, and then extracted with three 45 ml. portions of five percent aqueous sodium bicarbonate. The unnitrated starting material did not dissolve; the aqueous filtrate was acidified and cooled to 5° C. The product was filtered, washed with cold water and dried. The yield was 2.55 g.; M.P. 180—185° C., wet at 175° C. Two recrystallizations from 95% ethanol gave rosettes of pale yellow needles, M.P. 187—188° C.

*Analysis.*—Calcd. for  $C_{13}H_8O_7N_2$ : C, 51.32; H, 2.65; N, 9.21. Found: C, 51.41; H, 3.39; N, 8.55.

The same product (3.0 g.) was formed when 6.0 g. of 2,4-dihydroxybenzophenone was stirred for 2.5 hours with 120 ml. of 4 N nitric acid at 55—60° C.

The residues obtained by evaporating the ethanolic recrystallization liquors melted at 170—190° C. indicating a mixture. The nitrogen analysis (9.09%) was still consistent, however, with a dinitro-2,4-dihydroxybenzophenone.

3,3',5 - trinitro - 2,4 - dihydroxybenzophenone was prepared as follows: 2,4-dihydroxybenzophenone (10.7 g.; 0.05 mole) was added in small portions to 40 ml. of concentrated sulfuric acid ( $d=1.84$ ); the temperature was maintained at 10—15° C. by good stirring and cooling. Then 13 ml. of concentrated nitric acid ( $d=1.42$ ) was added dropwise during two hours while the temperature was held at 5—10° C. Near the end of the addition, solid began to separate. The nitration mixture then stood overnight at room temperature after which it was heated at 50° C. on the steam bath for 30 minutes. The recooled mixture was poured over 300 g. of crushed ice. The white solid which separated was removed by filtration, washed twice with cold water, and air dried; 17.6 g., M.P. 130—170° C. This impure product was fractionally crystallized from 95% ethanol. The first crop (5.8 g.) consisted of coarse, yellow needles which melted at 178—180° C.

*Analysis.*—Calcd. for a dinitro derivative  $C_{13}H_8O_7N_2$ : C, 51.32; H, 2.65; N, 9.21. Calcd. for a trinitro deriva-

5 *3* tive,  $C_{13}H_7O_9N_3$ : C, 44.71; H, 2.02; N, 12.03. Found: C, 45.59, 45.55; H, 2.21, 2.26; N, 12.12, 11.68.

These analyses indicate that the product is the trinitro-2,4-dihydroxybenzo-phenone contaminated with 12-14% of the dinitro compound.

Two other crops were recovered from the fractional crystallization: (1) 3.4 g., M.P. 168-173° C., N (found)=11.20%; (2) 2.3 g., M.P. 164-175° C., N (found)=10.77%.

*Example III*

3,5-dinitro-2,4 - dihydroxybenzophenone was dissolved in nitromethane at a concentration level of about two percent and the strand burning rate determined. The burning rate was increased 15-30 percent. Smooth burning was attained at 800 p.s.i.g. Substantially the same results were obtained using 3,3',5-trinitro-2,4-dihydroxybenzophenone as the additive.

*Example IV*

3,5-dinitro-2,4-dihydroxybenzophenone was dissolved in a 99% nitric acid-2-nitropropane system (stoichiometric to carbon dioxide and water) at a concentration level of two percent by weight. Strands were made from the composition and the strand burning rate determined. A burning rate increase of 50 percent resulted throughout the pressure range 100 to 300 p.s.i.g. Smooth burning and ignition were obtained down to 100-150 p.s.i.g., roughly 50-100 p.s.i.g. lower than for the mixture without ultraviolet light absorbers.

*Example V*

3,3',5 - trinitro - 2,4 - dihydroxybenzophenone was dissolved in the nitric acid-2-nitropropane system referred to above at a concentration level of two percent by weight and the strand burning rate determined. The results obtained were substantially the same as those obtained in Example IV.

A minor advantage of the polynitro-2,4-dihydroxybenzophenones as additives, over the unnnitroated compounds is the fact that they have a less negative oxygen balance and, therefore, do not require as much oxidizer for combustion. This advantage is especially important with nitromethane and other monopropellants which already have a deficiency of oxygen for combustion to carbon monoxide and water. Tests indicated that the optimum amount of ultraviolet light absorber is between about one and about ten percent by weight.

Ultraviolet light absorbers other than those used in the

examples may be used. It is only required that the absorber be soluble in the propellant and not react with it to cause propellant instability. Other nitroalkanes than those used in the examples may obviously be used and, particularly, the lower nitroalkanes. The nitroalkane selected will, of course, be that one which has the best overall properties as a propellant.

It is seen from the above description of the invention that it provides a simple method for increasing the burning rate and ease of ignition of liquid monopropellants derived from nitroalkanes. The additive is simply dissolved in the propellant or propellant system in the amounts disclosed and the propellant used in liquid propellant rockets of the type now well known in the art.

15 What is claimed is:

1. Liquid propellant compositions consisting essentially of a material from the class consisting of nitroalkanes and mixtures of nitric acid and nitroalkanes, said compositions being catalyzed by the addition thereto of not more than ten percent by weight of a substituted benzophenone having the formula:



wherein R is a member from the group consisting of alkoxy and hydroxyl, R' is a member from the group consisting of hydrogen, hydroxyl and alkoxy, R'' is a member from the group consisting of hydrogen and hydroxyl, and R''' is hydrogen or nitro.

2. The composition of claim 1 in which the substituted benzophenone is 2,4-dihydroxybenzophenone.

3. The composition of claim 1 in which the benzophenone is 2,2'-dihydroxy-4,4'-dimethoxybenzophenone.

35 4. The composition of claim 1 in which the benzophenone is 2,2',4,4'-tetrahydroxybenzophenone.

5. The composition of claim 1 in which the benzophenone is 3,5-dinitro-2,4-dihydroxybenzophenone.

6. The composition of claim 1 in which the benzophenone is 3,3',5-trinitro-2,4-dihydroxybenzophenone.

References Cited in the file of this patent

UNITED STATES PATENTS

|              |                      |                |
|--------------|----------------------|----------------|
| 45 2,433,943 | Zwickly et al. ----- | Jan. 6, 1948   |
| 2,537,526    | Hannum -----         | Jan. 9, 1951   |
| 2,542,193    | Hannum -----         | Feb. 20, 1951  |
| 2,853,522    | Dayan et al. -----   | Sept. 23, 1958 |